

Aug. 26, 1924.

1,506,104

E. R. WOLCOTT

PROCESS FOR PRODUCTION OF ALUMINUM CHLORIDE AND OTHER PRODUCTS FROM  
CARBONACEOUS SHALES AND LIKE MATERIAL

Original Filed Oct. 13, 1919 3 Sheets-Sheet 1



Aug. 26, 1924.

1,506,104

E. R. WOLCOTT

PROCESS FOR PRODUCTION OF ALUMINUM CHLORIDE AND OTHER PRODUCTS FROM  
CARBONACEOUS SHALES AND LIKE MATERIAL  
Original Filed Oct. 13, 1919 3 Sheets-Sheet 2

Original Filed Oct. 13, 1919 3 Sheets-Sheet 2



Aug. 26, 1924.

1,506,104

E. R. WOLCOTT

PROCESS FOR PRODUCTION OF ALUMINUM CHLORIDE AND OTHER PRODUCTS FROM  
CARBONACEOUS SHALES AND LIKE MATERIAL

Original Filed Oct. 13, 1919 3 Sheets-Sheet 3



INVENTOR

Edson R. Wolcott

BY

Arthur P. Knight

ATTORNEY

## UNITED STATES PATENT OFFICE.

EDSON R. WOLCOTT, OF LOS ANGELES, CALIFORNIA, ASSIGNOR, BY MESNE ASSIGNMENTS, TO THE TEXAS COMPANY, OF NEW YORK, N. Y., A CORPORATION OF TEXAS.

PROCESS FOR PRODUCTION OF ALUMINUM CHLORIDE AND OTHER PRODUCTS FROM CARBONACEOUS SHALES AND LIKE MATERIAL.

Application filed October 13, 1919, Serial No. 330,381. Renewed February 18, 1922. Serial No. 537,645.

To all whom it may concern:

Be it known that I, EDSON R. WOLCOTT, a citizen of the United States, residing at Los Angeles, in the county of Los Angeles and 5 State of California, have invented a new and useful Process for Production of Aluminum Chloride and Other Products from Carbonaceous Shales and like Material, of which the following is a specification.

10 This invention relates to the production of aluminum chloride and other products from materials containing aluminum silicate, and the main object of the invention is to provide for economical production of 15 aluminum chloride, or sodium aluminum chloride, by the utilization of carbonaceous argillaceous minerals, such as the so-called oil shales, or shales containing carbonaceous matter, as material for producing the aluminum compound and also for furnishing the 20 fuel required for the production of such compound. In this connection another object of the invention is to provide for the production of by-products from the carbonaceous constituent of the shale, and also in 25 some cases for the utilization of the carbonaceous constituent of the shale for other purposes, for example, for the production of power by combustion of certain of such 30 products.

The accompanying drawings illustrate more or less diagrammatically the apparatus suitable for carrying out the invention, and referring thereto:

35 Fig. 1 is a vertical section of the furnace or retort in which the shale or other aluminum-bearing material is treated, showing diagrammatically the connections therefor for treatment of the several products from such retort.

40 Fig. 2 is a view similar to Fig. 1 showing the connections required for production of special by-products from the carbonaceous or hydrocarbon constituent of the material being treated.

45 Fig. 3 is a view similar to Fig. 1 showing the connections required for carrying out the process when a halogen salt, such as sodium chloride, is used as the chloridizing 50 agent for treatment of the aluminum-bearing material.

My invention is particularly applicable to the production of aluminum chloride from carbonaceous shales, such as bituminous or oil shales, or other argillaceous materials 55 containing hydrocarbons or carbonaceous substances, and in this connection the invention will be described with particular reference to the treatment of oil shales so-called, that is to say, shales which upon destructive distillation yield more or less hydrocarbon or petroleum product. It will be understood, however, that the invention is applicable to other clay substances, such as argillaceous fuels including slaty coal, or 60 shale containing coal, impure or low grades of lignite or coals, and generally to any material containing alumina or aluminum silicate and carbon or carbonaceous material. The invention contemplates the treatment of 65 a carbonaceous argillaceous mineral, comprising alumina or aluminum silicate and carbonaceous material, of such nature as to be capable of yielding on heating or distillation vaporous hydrocarbon products and a residue containing carbon and aluminous material adapted for reacting with added chlorine to form aluminum chloride.

The apparatus shown on the drawing in Fig. 1 comprises a retort 1 formed, for example, as a vertical cylinder of suitable material having an inlet 2 at its upper end through which the material to be treated is fed into the retort and an outlet 3 at its lower end through which waste material 75 may be drawn. Suitable means, such as a hopper 4, provided with feed means, not shown, may be provided at the upper end of retort 1 for feeding into the retort 1 the oil shale, or other material, after same has been 80 crushed or reduced to a suitable size by a crusher indicated at 5.

The retort 1 is surrounded by a casing or enclosing means 7 forming a combustion and heating chamber 8 around said retort, said chamber being heated by suitable burner means indicated at 9 and having an outlet 10 at its upper end for the products of combustion. Two pipe lines or conduits 11 and 12 lead from the upper part of retort 1, 95 said pipe lines or conduits being provided with valves or dampers 13 and 14 whereby

they may be opened alternately, as herein-after set forth.

- The pipe line 11 is for conducting away the hydrocarbons, or other carbonaceous gases and vapors produced by the destructive distillation of the oil shale and may be connected to a condenser 15 and means 16 for receiving the condensed products. A connection 17 having a pump 18 may be provided for drawing uncondensed gases and vapors from the receiving means 16 or from the pipe line 11 and forcing same into a suitable means, such as a gasometer or gas reservoir 19 for storing such gases or vapor products of the distillation. A pipe connection 20 may lead from this storage reservoir to the burner 9 so as to heat the oil shale by combustion of the gas derived from destructive distillation thereof.
- Pipe line 12 leads through a condenser 22 to suitable filter or precipitator means 23 for removing from the gases passing thereto the material condensed in the condenser 22.

The device 23 is shown as a filter chamber having a filter wall 24 through which the gases are drawn by pumping means 25, the condensed product, which is in general solid at the temperature of operation, running down into a collecting chamber 26 or being removed thereinto by suitable means 27.

Receiver 26 is shown as provided with an outlet 28 for the collected material and with another outlet 29 leading to a purifying apparatus shown as a revolving drum 30 in the furnace chamber 31 heated by burner means 32, said revolving drum opening into a settling chamber 33 from which a conduit 34 leads to a filter or precipitator 35. From said filter or precipitator a connection 36 conducts the filtered or precipitated material to a storage tank 37. From said tank the material may pass through one or more of several different operations, as herein-after described, according to the product which it is desired to produce.

The process may be carried out in the above described apparatus in the following manner: The oil shale or similar material is passed through the crusher 5 so as to be reduced to a suitable state of division, preferably in the form of lumps or fragments sufficiently small to present a large surface to the heating action and sufficiently large to enable free passage of the chloridizing gases through and free delivery of the volatilized vapors from the material. For this purpose the material may be crushed to, say, one-half inch mesh or thereabout. The material is supplied through the inlet tube of the retort 1 until said retort becomes charged and the upper end of the retort may then be closed by a suitable lid or cap extending, for example, over the top of the hopper 4 so that the retort becomes substantially

sealed from admission of outside air. The heating chamber 8 is then heated in any suitable manner, for example, by combustion of fuel supplied through pipe 40 and air supplied through opening 21, damper 14 being closed and damper 13 being open the first stage of the distilling operation proceeds in the following manner:

The oil shale becomes heated by conduction of heat through the walls of conduit 1, resulting in destructive distillation thereof and the volatilization of carbonaceous vapors, mainly hydrocarbons, which pass off through pipe 11 and are cooled in condenser 15 so as to liquefy the more condensable constituents thereof, forming oils which collect in receptacle 16, the residual gas and vapors being drawn off to the storage tank 19. When sufficient combustible gas has been accumulated in this manner in the storage tank 19, a portion thereof may be drawn through outlet pipe 20 to the burner 9 for continuing the heating of the retort 1. Any excess of gas not required for this purpose may be delivered to any other desired consuming device by branch pipe 42. For example, it may pass to a power plant, indicated at 38, using hydrocarbon for the generation of power to operate a dynamoelectric generator 39, which supplies current through leads 49 to an electric furnace 50 used in connection with the process. The oil accumulating in the receptacle 16 may, if desired, be passed off through pipe 43 and treated in any suitable manner (in refining or distilling apparatus indicated at 41), if desired, for producing one or more commercial products, or such oil, or the residuum after such treatment, may be passed to a burner 44 for assisting in the heating operation in the combustion chamber 8. Any valuable hydrocarbon by-products produced in the apparatus 41 may be led off by pipe 39 and utilized in any suitable manner. Or, if desired, part or all of the oil or liquid hydrocarbons produced from the condenser 15 may be drawn off through pipe 43' for use or sale as such.

When the destructive distillation of the carbonaceous content of the oil shale has been completed by the above described operation (which will, in general, be determined by the cessation of flow of the hydrocarbon gases and vapors through the pipe line 11), the said pipe line is closed by damper 13 and damper 14 for the pipe line 12 is then opened and the process then passes to the second stage of distillation which consists in a chloridizing volatilization of the aluminum content of the clay. In this connection, it is necessary to use a chloridizing agent, or volatilizing agent, and for this purpose I prefer to use gaseous chlorine introduced through the inlet 46, which opens into the outlet 3 of the retort 130

1. Immediately following the completion of the first or destructive distillation and while the residual material in the retort is still hot, the chlorine is turned on or admitted through the pipe 46 from any suitable source, indicated as a storage tank 48, and the heating is continued, the retort 1 being maintained at a suitable temperature by continued admission of fuel to one or more of the burner means 9, or 44, aforesaid. The aluminum silicate present in the clay or shale residue is in intimate contact with carbon distributed throughout the mass of said clay or shale, such carbon being the residuum from the destructive distillation of the carbonaceous content of the clay or shale. The fragments of clay or shale are also in contact with chlorine passing upwardly through the retort 1. Under the action of the heat maintained in said retort and in the presence of the said carbon and chlorine, the action takes place in such manner that aluminum chloride is produced, and being volatile at the temperature of operation passes off through the pipe line 12. Passing through the condenser 22 the aluminum chloride is condensed from the fume, which is collected in the filter or precipitator 23, passing therefrom to the receptacle 26. The aluminum chloride so collected will generally be in the form of a fine powder containing more or less impurities, especially ferric chloride, derived from impurities in the original clay or shale. In some cases, however, the product may be sufficiently pure for use and sale as commercial aluminum chloride and may be withdrawn for that purpose through outlet 28.

40 In case further purification is desired the aluminum chloride may be passed through conduit 29 to the re-volatilizing drum 30, wherein it is subjected to sufficient heat to volatilize the aluminum chloride, while leaving other materials, for example, ferric chloride, in un-volatilized condition. Such other materials pass out as waste, as indicated at the lower end of the drum 30. The vapor of aluminum chloride issuing from the drum 30 passes through chamber 33 wherein any dust passing over with same is settled out and then passes to the filter or precipitator 35, which collects the fume of the condensed aluminum chloride and discharges the same into the storage tank 37. Aluminum chloride so produced may be used or sold for use for ordinary commercial purposes, for example, as an agent in petroleum refining. It may, however, if desired, be used for production of metallic aluminum, and in that case aluminum chloride from the receptacle 37 may be electrolyzed in the electric furnace 50 to produce metallic aluminum and chlorine (the latter being delivered to tank 48 aforesaid), or, if

it is desired to produce alumina for use in aluminum production, aluminum chloride from the receptacle 37 may pass to a hydration tank 52 wherein it is brought into contact with water so as to form aluminum 70 hydrate and hydrochloric acid, which are then heated in the heater 53 so as to produce anhydrous alumina and to drive off the hydrochloric acid gas, which may be sold or utilized as such, or may pass 75 through a catalytic chamber 55 wherein it is brought in contact with a suitable catalytic agent, such as heated cupric chloride, in the presence of oxygen or air introduced at 59 to produce water and chlorine. The 80 water is removed in the condenser or dehydrator 57 and the free chlorine passed to tank 48. Any chlorine required in the process, in addition to that recovered from the above described operations, may be supplied 85 from any suitable source.

In the above described embodiment of my invention, the carbonaceous or hydrocarbon products of the first distillation are utilized both for heat production and for power 90 generation in connection with the process, and any surplus of power or of fuel may be utilized in any suitable manner. It will be understood that in order to provide for continuous operation, duplicate retorts 1 may 95 be provided and operated alternately so that one retort may be always in condition to deliver fuel for the stated purposes. If desired, however, this can be provided for by making the storage means 16 and 19 of sufficient capacity. In special cases it may be desirable to use a major part of the fuel products of the process in the production of power, and in case the power plant is adapted to use the crude product, the latter may 100 be led directly to said plant from the pipe 11.

105 In many cases the amount of carbonaceous material contained in the clay material under treatment is not sufficient to provide the fuel required for distillation purposes or the fuel required for power generation in connection with the process, or for both of such purposes, and, in such cases, it is desirable to subject an additional quantity 110 of the carbonaceous or oil shale, etc., to suitable treatment, for the production of fuel therefrom; for this purpose such additional quantity of the oil shale may (either with or without preliminary heating in any suitable retort to first drive off the hydrocarbons, which may be utilized as above described) be subjected while at high temperature to the action of steam or of air, or both, to make producer gas, the resultant gases being 115 introduced into the combustion chamber of the retort 1, or into the combustion chamber of the power generating plant or apparatus 38, for the generation of electrical current 120 for use in connection with the process and, 125 in such cases, the amount of additional oil 130

shale, or carbonaceous shale, or low grade coal, used in this manner is not necessarily limited to what is required for carrying out the distilling operations aforesaid and for 5 producing the power for electrolysis in connection with the above described process, but may be made as auxiliary to or in connection with a power plant for general power generating purposes. This treatment 10 of additional oil shale, etc., for the production of additional fuel may be carried out in an auxiliary retort or producer indicated at 58, discharging by the pipe 59 to pipe 20 leading to the combustion chamber 15 8 and by pipe 59' to the power plant 38.

In some cases it may be desirable to utilize the hydrocarbon products of the destructive distillation of the oil shale, etc., in the production of valuable by-products. In this 20 connection, the chlorine supply provided in connection with the second stage of distillation may be advantageously utilized in the formation of such by-products, the hydrocarbons being subjected to the action of 25 such chlorine to produce substitution or addition products, as may be desired. A flow sheet for such an embodiment of my invention is shown in Fig. 2 wherein the retort and the two pipe line connections therefrom 30 are similar to those shown in Fig. 1, but there is provided in addition a catalyzing chamber 60 adapted to receive hydrocarbon gas or vapor from a suitable part of the connections to pipe line 11 (for example, from 35 gas holder 19), and to also receive chlorine from a connection 64, said catalyzing chamber being provided with means such as a jacket 76 provided with piping 77 for passing a heating medium therethrough for 40 maintaining the proper conditions of temperature to cause reaction of the chlorine with such hydrocarbon to produce the desired chlorinated hydrocarbon product. As an illustration, the process may be used to 45 produce carbon tetrachlorid, ethylene dichlorid, or other substitution or addition products, which constitute commercial products and may be sold as such, or may be used for production of other hydrocarbon derivatives. These products may be discharged 50 through pipe 61 to a separator 73 from which the residual gases, including residual hydrocarbon gases pass by pipe 74 to combustion chamber 8.

55 The chlorine required for the process may conveniently be produced by electrolysis of sodium chloride in an electrolyzer 63, the chlorine passing to the drier 65 and then by pipe 64 to the catalyzing chamber 60, and by pipe 62 to the chlorine inlet 46 of the retort 1. The sodium hydrate from the electrolyzer 63 may pass through the stages of evaporation and fusion as indicated to 60 form a commercial product.

65 In treating the product of the second dis-

tillation (consisting essentially of aluminum chloride) for the production of aluminum, I may first convert the aluminum chloride to alumina, as above described and as indicated at 52, and then electrolyze such alumina in 70 an electric furnace, as indicated at 66 in Fig. 2. The hydrochloric acid produced in tank or chamber 52 may be decomposed in electrolyzer 67 to produce chlorine, which is returned by pipe 68 to drier 65 and hydrogen, which may be used for hydrogenation, in an apparatus indicated at 69, of one or more of the hydrocarbon derivatives produced from the products of the first distillation. Similar disposition may be made of 80 the hydrogen from the electrolyzer 63. Or the hydrogen can be compressed and sold as a commercial article.

In some cases, I may use sodium chloride, or an equivalent salt, instead of gaseous chlorine as a chloridizing agent in the second distillation, the sodium chloride, or other salt, being introduced at 70, as shown in Fig. 3, into the retort 1, and the volatilized product in that case being mainly a double 85 chloride of sodium and aluminum. This double salt may be purified, if necessary, in apparatus 30', and then electrolyzed in an electric furnace 71, producing metallic 90 aluminum and gaseous chlorine. Such 95 chlorine is advantageously returned to the retort 1, as it is desirable to furnish a certain amount of free chlorine, together with the sodium chloride, to ensure effective volatilization of the sodium-aluminum chloride. The operation may be otherwise carried out in the same manner as described in connection with Fig. 1 or Fig. 2.

In any of the above described embodiments of my invention, the waste or residual material from the final distillation and consisting mainly of siliceous gangue, is withdrawn at the end of the operation through outlet 3 and the retort 1 then charged with fresh material for repetition of the operation.

In general the shale to be treated contains considerable water and, in case it is desired to eliminate this before the first distilling operation, the water vapor may be carried off through a pipe 21<sup>a</sup>, see Figs. 1, 2 and 3, so as not to mix with the hydrocarbon products. In case the clay used contains an appreciable amount of iron, this may be eliminated by passing hydrochloric acid through gas inlet 46 into the retort 1, after the water has been eliminated and preferably after the hydrocarbons have been distilled off. By passing hydrochloric acid in contact with dry clay at a suitable temperature, say about 900° C., I am enabled to drive off all the iron as a volatile compound, leaving the aluminum compound mainly unaffected, so that in the ensuing or final distillation aluminum chloride is produced in 130

pure condition. The same operation may be effected by passing hydrochloric acid from stage 52 (in Fig. 2) to retort 1.

As an alternate method of freeing the alumina produced by my process from iron and other impurities, I may treat the alumina (produced at stage 52 in Figs. 1 and 2) with caustic soda solution to form aluminate, and then precipitate the alumina by reaction with alumina or with  $\text{CO}_2$  in well known manner, or other methods of purification may be used.

What I claim is:

1. The process of making aluminum chloride comprising reacting with a chloridizing agent upon a distillation residue derived from carbonaceous shale, said residue comprising aluminum silicate having carbon intimately associated therewith.

2. The process which consists in subjecting a carbonaceous argillaceous mineral to heat to effect destructive distillation in such manner as to volatilize hydrocarbon compounds, then, while maintaining the material in heated condition, introducing a chloridizing agent into contact with said material, to heat to volatilize and drive off aluminum chloride, and collecting said aluminum chloride.

3. The process which consists in subjecting carbonaceous shale to heat to effect destructive distillation to volatilize and drive off hydrocarbon compounds and to leave residual carbon in the material being treated, then while continuing the heating operation introducing chlorine into contact with the residual material and subjecting the material to further distillation to volatilize aluminum chloride, and collecting said aluminum chloride.

4. The process which consists in subjecting a carbonaceous argillaceous mineral to sufficient heat to drive off hydrocarbons leaving residual carbon in the material, then introducing a chloridizing agent to the residual material and subjecting the same to further heat to volatilize a compound of aluminum and chlorine, condensing said compound of aluminum and chlorine and recovering the same separately from the hydrocarbon compound aforesaid.

5. The process which consists in subjecting material containing a carbonaceous argillaceous mineral to a drying operation to remove moisture therefrom, then to heating operation sufficient to volatilize hydrocarbon compounds from the carbonaceous material, then introducing hydrochloric acid and continuing the heating at sufficiently high temperature to volatilize as ferric chloride any iron present in the residual material, and then passing chlorine into the residual material containing aluminum silicate and residual carbon and subjecting the material to heat to produce and volatilize aluminum

chloride, and collecting such aluminum chloride.

6. The process which comprises subjecting to heat a carbonaceous argillaceous mineral to effect destructive distillation in such manner as to volatilize and drive off hydrocarbon compounds, leaving a residual material containing aluminum silicate and residual carbon in intimate association, subjecting the residual material to heat in the presence of a chloridizing agent to produce and volatilize aluminum chloride, condensing and collecting the aluminum chloride with such impurities as may be contained therein, purifying the aluminum chloride by subjecting it to sufficient heat to revolatilize the aluminum chloride, and finally collecting the aluminum chloride in a pure state.

7. The process which comprises preliminarily crushing a carbonaceous argillaceous mineral, heating this crushed material in a closed retort out of contact with the air to volatilize and drive off any moisture contained therein, continuing the heating of the dehydrated material to volatilize and drive off the hydrocarbon compounds thereby leaving a residual material containing aluminum silicate and residual carbon in intimate association, contacting the residual material with a chloridizing agent while continuing the heating operation to produce anhydrous aluminum chloride in a volatile state.

8. The process of making aluminum chloride comprising reacting with chlorin upon a residue derived from heating a carbonaceous argillaceous mineral, said residue comprising aluminous material and carbon.

9. The process of making aluminum chloride comprising contacting a chloridizing agent with a heated residue derived from a carbonaceous argillaceous mineral.

10. The process of making aluminum chloride that comprises heating a carbonaceous argillaceous mineral containing aluminous material and carbon in intimate association and contacting said mineral with a chloridizing agent.

11. The process of making aluminum chloride that comprises heating material comprising a carbonaceous argillaceous mineral containing aluminum silicate and carbon in intimate association and introducing a chloridizing agent into contact with said mineral.

12. The process of making aluminum chloride that comprises reacting with a chloridizing agent upon a residue derived from heating an argillaceous fuel.

13. The process that comprises subjecting a carbonaceous argillaceous mineral to heat to drive off hydrocarbon products, contacting the residual material with a chloridizing agent while applying heat to produce alumini-

num chloride vapors, condensing and collecting the aluminum chloride thus produced, treating said aluminum chloride electrolytically to produce aluminum and chlorin and passing said chlorin and aforesaid hydrocarbon products in contact with heated catalytic material to form chlorinated hydrocarbons.

14. The process that comprises subject-  
10 ing a carbonaceous argillaceous mineral to heat to drive off hydrocarbon products, contacting the residual material with a chloridizing agent while applying heat to produce aluminum chloride vapors, condensing  
15 and collecting the aluminum chloride thus produced, hydrolyzing said aluminum chloride to form hydrated alumina and HCl, treating said products electrolytically to produce aluminum from said alumina and  
20 hydrogen and chlorin from the HCl and contacting said hydrogen with aforesaid hy-

drocarbon products under conditions to form hydrogenated products.

15. The process that comprises heating a carbonaceous argillaceous mineral to drive 25 off hydrocarbon vapors and obtain a residue comprising an aluminous material and carbon, treating a solution of sodium chloride electrolytically and introducing the chlorin derivative of the electrolysis into contact 30 with said residue while applying heat to same to generate aluminum chloride vapors, collecting said aluminum chloride and passing the hydrogen derivative of aforesaid electrolysis into contact with aforesaid hydrocarbons under conditions to form hydrogenated products.

In testimony whereof I have hereunto subscribed my name this 6th day of October 1919.

EDSON R. WOLCOTT.